

[54] PROCESS FOR PRODUCING TEXTURED YARN

[75] Inventors: Brewster B. Eskridge; Roger H. Fink; William D. Porter, all of Asheville; Elbert K. Warren, Candler, all of N.C.

[73] Assignee: Akzona Incorporated, Asheville, N.C.

[21] Appl. No.: 681,252

[22] Filed: Apr. 28, 1976

Related U.S. Application Data

[62] Division of Ser. No. 517,802, Oct. 24, 1974, Pat. No. 3,983,610.

[51] Int. Cl.<sup>2</sup> ..... D02G 1/12; D02G 1/16

[52] U.S. Cl. ..... 28/221; 28/255

[58] Field of Search ..... 28/1.3, 1.4, 1.6, 1.7, 28/72.11, 72.12, 72.14, 221, 255

[56] References Cited

U.S. PATENT DOCUMENTS

|           |         |                    |        |
|-----------|---------|--------------------|--------|
| 3,343,240 | 9/1967  | Parmeggiani et al. | 28/1.3 |
| 3,409,956 | 11/1968 | Longbottom et al.  | 28/1.3 |
| 3,559,254 | 2/1971  | Stanley            | 28/1.6 |
| 3,693,222 | 9/1972  | Caffry             | 28/1.6 |
| 3,707,745 | 1/1973  | Nikkel             | 28/1.3 |

|           |         |                 |          |
|-----------|---------|-----------------|----------|
| 3,810,285 | 5/1974  | Ferrier et al.  | 28/1.3 X |
| 3,824,656 | 7/1974  | Bauch           | 28/1.3   |
| 3,840,950 | 10/1974 | Stanley         | 28/1.3   |
| 3,852,857 | 12/1974 | Ethridge et al. | 28/1.3   |
| 3,895,420 | 7/1975  | Sturtz et al.   | 28/72.14 |

FOREIGN PATENT DOCUMENTS

861,327 2/1961 United Kingdom ..... 28/72.12

Primary Examiner—Robert R. Mackey  
Attorney, Agent, or Firm—Craig & Antonelli

[57] ABSTRACT

Multifilament synthetic polymer yarn is texturized by passing the yarn in a gas stream to a diffuser zone to cause the gas to expand and the yarn filaments to splay open. The yarn filaments are then separated from the expanding gas stream towards a continuous smooth side wall surface defining one end of a bulking chamber. At this end of the chamber the filaments are impacted with each other and the smooth wall surface to form a compact yarn mass. This yarn mass is pushed into and through a slotted portion of the bulking chamber. Simultaneously the gas passes through the yarn mass initially formed in the chamber and then discharges laterally from this mass as it is pushed into the slotted portion.

13 Claims, 7 Drawing Figures



FIG. 1.



FIG. 2.



FIG. 3.



FIG. 4.



FIG. 5.



FIG. 6.



FIG. 7.



## PROCESS FOR PRODUCING TEXTURED YARN

CROSS-REFERENCE TO RELATED  
APPLICATION

This application is a division of application Ser. No. 517,802 filed Oct. 24, 1974, now U.S. Pat. No. 3,983,610.

## BACKGROUND OF THE INVENTION

This invention relates to the production of texturized yarns or like multifilament groups of synthetic polymeric materials, e.g. tows, and more particularly to an apparatus and process for texturizing yarn to provide uniform random crimps in the filaments of the yarn by pneumatically conveying the yarn into a bulking chamber to form an elongated uniformly compacted yarn mass and to the yarn products resulting from the process.

Heretofore, many apparatus and processes have been developed for texturizing yarn made of thermoplastic polymeric materials by the use of fluid jets or like pneumatic means. Many of these prior developments have been relatively successful in providing bulky voluminous yarn having a degree of crimp uniformity and improved dyeing characteristics suitable for use in the production of textile fabrics, carpets and the like. However, the apparatus employed for carrying out many of these known processes is complex and requires elaborate machining techniques to produce. This apparatus is costly and for this reason less elaborate and slower stuffer box crimping systems, wherein relatively straight feeder yarn is forced into a compression chamber by a pair of driven rolls and is accumulated within the chamber by pressure developed within the chamber, are often employed. In these systems the feeder yarn forms wads of yarn in the compression chamber and a regular crimp is imparted to the individual filaments of the yarn during this accumulation. Also heated fluids such as steam or hot air are often utilized to moisten and/or heat-set the yarn while in a crimped state within the compression chamber.

Because of the advantages found in the yarns produced by the pneumatic bulking or texturizing systems, particularly the high yarn processing speeds, and random crimping of the filaments, the difficulties in producing the necessary apparatus as well as the complex controls required for operating such apparatus have been accepted by the industry. In these known processes an initially straight and pre-drawn yarn which may be untwisted or slightly twisted is subjected to a turbulent fluid, such as steam, in such a manner that the individual filaments of the yarn are looped, coiled, or crimped and the yarn is heat-set in this condition. The individual filaments are in this manner formed into a bulky wool-like product wherein each of the filaments in a relaxed condition exhibit a plurality of crimps or loops along a given length. These crimps are usually offset and out of phase with each other in a random manner.

One difficulty encountered in these known pneumatic processes is a requirement to provide a sufficient number of crimps to a given length of yarn. Often it is difficult to obtain consistently more than 10 crimps per inch in the filaments of the resulting yarn product.

Many prior attempts to improve the crimp count involve procedures to impinge, fold or coil the yarn in such a manner that the yarn filaments are highly crimped while allowing the yarn to be subsequently

removed from the apparatus without loss of desired yarn properties.

Also, the procedures used for separating the yarn from the fluid stream, usually hot air or steam, are important to the success of the crimping process. Various devices such as angled baffles, bulking tubes with reverse exhaust, bulking chambers with lateral exhaust ports, rotating screen drums and the like have been employed. The use of such devices often imposes limitations of yarn speed, yarn uniformity or process flexibility on the known processes.

In order to overcome a number of drawbacks attendant to these pneumatic bulking techniques, several developments have been made. For example, U.S. Pat. No. 2,982,082 discloses a process and apparatus for producing luminous yarn wherein a continuous filament yarn is fed into a jet by a pair of rollers. The jet has an inlet tube extending through a chamber and is provided with a jet tip which faces and enters the mouth of a venturi passage. The outer surface of the jet and the mouth of the venturi cooperate to form an annular passage for a fluid stream under pressure to be blown into the chamber and out through the venturi. The yarn is drawn out of the jet by an additional pair of rollers at such a rate that the yarn is overfed to the jet so that the individual filaments of the yarn are formed into loops and curls by the turbulence of the air stream beyond the annular passage within the jet.

U.S. Pat. No. 3,373,470 describes a process for stuffer-type crimping of thermoplastic filaments wherein the filaments are introduced into one end of an elongated confined space by a stream of fluid such as steam under pressure and at a temperature sufficient to set the filaments. The filaments are tightly packed within the confined space by controllably releasing part of the fluid from the confined space laterally of the confined space at a position spaced from the other end and the packed filaments are then forced through the space to the other end under pressure by the remaining portion of the fluid which exhausts with the yarn. The confined space required for this process is defined by a metal spring having gaps between the convolutions thereof. In this apparatus the yarn is propelled by the action of the fluid from a nozzle through a tubular passage and then into the interior of the spring. The spring is curved to a desired extent to obtain optimum packing of the yarn therein.

U.S. Pat. No. 3,380,242 describes yet another process for providing a crimp to synthetic yarns wherein the yarn is subjected to the action of a turbulent stream by passing it through a jet to which a hot gas is supplied. The yarn and hot gas leaving the jet enter a venturi tube wherein the individual filaments of the yarn while in a plastic state and under substantially zero tension are separated from each other and crimped individually while whipping about in the turbulent plasticizing stream. The crimp produced by this process has a random three-dimensional curvilinear extensible configuration.

There are still a number of drawbacks, such as uneven or irregular dyeing characteristics, non-uniform crimping and the occurrence of snarls or tangles in the yarn which need to be overcome. For example, in the manufacture of tufted carpets it has been found that tufting machines require particularly uniform yarns and that snarled yarns will cause stoppage, broken filaments and even end breakage. Also, the snarled or tangled yarn will provide faults in the carpet product. There-

fore, manufacturers of texturized carpet yarns are continuously looking for apparatus and processes to provide bulky yarns which will dye uniformly and which are free from snarls and tangles.

#### SUMMARY OF THE INVENTION

Advantageously, the present invention provides a continuous pneumatic process that produces bulky yarns having a high degree of random crimp and that can be carried out at high speeds by an apparatus which is simple to manufacture and which can be operated without elaborate controls. Furthermore, the dense yarn mass produced during the process of this invention is characterized by a symmetrical compact arrangement of the filaments which enables the yarn to be easily removed from the apparatus. This yarn mass provides a bulky yarn product that has a highly uniform and even random crimp in each of the filaments and that is substantially free of snarls and tangles.

This invention contemplates a process for texturizing or bulking a multifilament synthetic polymeric yarn wherein the yarn is passed in a gas stream to a diffuser zone to cause the gas to expand and the yarn filaments to splay open; the yarn filaments are directed away from the expanding gas stream towards a continuous smooth side wall surface defining one end of a bulking chamber; the filaments are impacted with each other and the smooth side wall surface to form a compact yarn mass at the one end of the bulking chamber; and the yarn mass is pushed into and through a slotted side wall or otherwise gas permeable portion of the bulking chamber; while the gas simultaneously passes through the yarn mass initially formed at one end of the bulking chamber and then discharges laterally from the yarn mass pushed into the slotted portion of the bulking chamber.

In this process, the yarn is initially delivered at a constant speed by a feeding device such as feed rollers, godet or the like to a bulking jet. Delivery yarn speeds of from 500 to 2,000 meters per minute may be used; preferably the speeds are from 1,000 to 1,500 meters per minute. Prior to entering the bulking jet, the yarn is preheated to 100° C to 200° C. by a plate heater, godet or like heating device or in some cases, the yarn is heated by being drawn immediately before entering the bulking jet.

The yarn is then aspirated into the bulking or aspirator jet by the venturi effect of a heated gas, such as superheated steam or compressed air. The yarn carried in the gas stream then enters a preheat tube where the yarn temperature is raised by the heated gas to plasticize the yarn prior to crimping and/or folding in the bulking chamber. In the preheat tube, the yarn is heated to temperatures between the second order transition point and the melting point of the yarn; the temperature of the yarn is maintained below the sticking point to avoid the formation of separate coherent filament groups within the yarn.

The yarn and gas stream exit from the preheat tube into a diffuser zone having a diverging conical wall surface. In this zone, the gas is expanded very rapidly to create great turbulence, thereby causing the yarn filaments to splay open, to flutter violently, and to move towards the conical wall surface. Folding-over of the yarn filaments occurs as the filaments impinge against each other and a smooth side wall surface of a plug forming zone of the bulking chamber immediately adjacent to and downstream from the diffuser zone. Conse-

quently, the yarn accumulates at the front end of the bulking chamber to form a compacted mass in the form of an elongated, cylindrical plug which seals off the downstream end of the bulking chamber. Further accumulation of yarn and the force of the entering gas cause the accumulated yarn plug to be pushed forward into a slotted wall portion of the bulking chamber while the yarn newly entering the chamber impinges at random on the upstream end of the dynamically forming plug in the plug forming zone. All of the gas from the diffuser zone now flows through the compacted yarn mass at the front end of the bulking chamber and after reaching the slotted portion of the bulking chamber, the gas exhausts laterally from the yarn plug. In this manner, the yarn in the smooth wall portion is uniformly treated with the gas to cause crimping and bulk-setting of the yarn.

The yarn filaments, which fold upon each other and themselves and on the smooth side wall surface, are, generally, arranged at an angle to the longitudinal axis of the bulking chamber (as well as the coinciding longitudinal axis of the plug) with intermediate portions forming successive inwardly and outwardly curved folds, or pleats much like those of an accordion. The filaments appear to splay open and then close together in a pulsating manner during formation of the plug. The filaments converge initially form a concave surface towards the downstream end of the chamber upon which subsequent filaments are compacted. This arrangement causes the filaments to be built-up in a conical-like stacked arrangement within the bulking chamber. Generally, the major portions of the filaments form an angle with a plane perpendicular to the longitudinal axis of the chamber that may vary from about 10 to 30°. Also, the smooth side wall surface provides an ironing-effect on the outer surface of the plug. Consequently, when the plug moves forward in the bulking chamber and when the steam exhausts through the slots or perforations in the bulking chamber, yarn is not carried out with the gas which would cause large loops, snarls and other variations in the yarn crimp.

The continuous multifilament yarns to be texturized by this invention are made from various thermoplastic synthetic polymeric materials such as nylon; polyester, e.g. polyethylene terephthalate; polyolefins, e.g. polypropylene; acrylic polymers, e.g. polyacrylonitrile and copolymers of acrylonitrile; polyvinyl chloride, polyphenylene oxides and other fiber-forming materials. Preferably, the yarns used for the purposes of this invention are those made entirely of nylon or polyester. However, yarns made of composite filaments such as nylon and polyester may also be employed.

The denier of the feeder yarns utilized in the practice of this invention may vary from about 50 to 4,000 and the denier used for producing carpet yarns usually varies from about 1,000 to 3,000. These yarns, which are drawn prior to bulking, include twisted or untwisted flat yarn as well as spin-drawn yarn, spun yarn which is subsequently drawn, and the like yarns. Also, the yarn may be drawn immediately before being introduced into the bulking jet. In general, the yarn is drawn at conventional draw ratios employed for orientation of synthetic polymeric filaments prior to crimping, e.g. 2.5 : 1 to 4 : 1; with a draw ratio of 3.6 : 1 being particularly effective for nylon carpet yarns. Partially drawn feed yarns produced from high speed filament spinning may also be utilized, in which case draw ratios before the

bulking jet will be proportionately lower during the additional drawing.

The feeder yarn usually will have selected oil and/or emulsion finishes applied thereto to achieve a proper moisture and finish content.

It has been found that the gas used to aspirate the yarn in accordance with this invention advantageously is a dry gas such as superheated steam or compressed air. Preferably, superheated steam is used. This steam has a pressure of from about 50-100 psig, and a temperature from about 200° C. to about 275° C. The preferred pressure for nylon 6 carpet yarns is from 60 to 80 psig, and preferred temperature is from 220° C. to 240° C. Usually the temperature of the steam is above the melting point of the yarn since heat losses in the system and the short residence time of the yarn with the steam prevent the yarn from being raised to this melting temperature.

Air suitable for purposes of this invention can be taken from the atmosphere at ambient conditions and compressed to 50 - 100 psig, and heated to 200° to 275° C.

After the yarn plug has been pushed from the bulking chamber, the yarn plug, while still intact, is guided through a tubular conduit to a plug guide where the 25 yarn is removed from the plug by a takeup device at a rate that is about 15-25% slower than the feed rate. Sufficient tension is applied to the yarn to cause it to stretch out to a length less than the original length, and to pull the filaments back into a yarn bundle.

Optionally, the yarn may be passed through a tangle jet for additional bulk control to establish desired yarn properties and then through a steam annealing jet before winding into a take-up package. U.S. Pat. No. 3,461,521 discloses specific annealing and air tangling 35 means that can be utilized.

This invention is also directed to an apparatus for effecting the heretofore described bulking process, which apparatus comprises: (1) a pneumatic aspirator jet having an inlet means for supplying a heated gas to 40 a jet orifice for producing a gas stream within the aspirator, and a yarn inlet means for introducing a yarn into the gas stream; (2) a preheat tube secured to the aspirator jet defining a narrow passage for receiving the yarn carried by the gas stream and for allowing the yarn to 45 be preheated by the gas; (3) a diffuser having a conical diverging surface at the end of said preheat tube; and (4) a bulking chamber adapted to contain a compacted yarn mass therein, said chamber having a smooth side wall portion adjacent to the conical surface of the diffuser for forming the compacted yarn mass and a slotted wall portion for receiving the compacted yarn mass and for discharging gas laterally from said yarn mass.

Advantageously, the position of the front of the plug within the bulking apparatus of this invention remains substantially constant. However, the invention also contemplates control means for regulating the position of the compacted yarn mass, i.e. the yarn plug in the bulking chamber. More specifically, it has been found that the position of the plug is dependent on the temperature and/or pressure of the entering heated gas as well as the temperature of the preheated feeder yarn. Yarn sensing means can be placed in the bulking chamber to determine the position of the initially formed plug. When this portion of the plug is displaced from the smooth wall portion of the bulking chamber onto the slotted portion, the temperature and/or pressure of the gas is decreased sufficiently to cause the yarn plug to

return to its proper position on the front smooth wall portion. Likewise, displacement of the plug into the diffuser can be corrected by increasing the temperature and/or pressure.

5 In another system of the invention, the plug within the bulking apparatus can be controlled by regulating the position of the end of the plug pushed out of the apparatus. The plug is moving at a rate on the order of 1/200th of the yarn input rate in the conduit or like 10 means for guiding the yarn. The plug is directed into a plug guide wherein an accumulator device or yarn sensing means, e.e. feeler elements, contact the yarn. When the plug moves past a predetermined set point, the yarn feeler element closes a switch and thereby causes the apparatus to shutdown. If the yarn recedes toward the inlet of the plug guide and accumulator device, another feeler element and associated switch are actuated to cause shutdown. Between these positions, additional sensing means can be used to regulate the speed of the take-up device. A control device of this type is further described in the application of Roger H. Fink et al. executed on even date herewith Ser. No. 517,786 filed Oct. 24, 1974).

The process and apparatus of the invention will be further understood from the following detailed description and the accompanying drawings wherein:

FIG. 1 is a sectional view of a preferred embodiment of the apparatus for texturizing a yarn according to this invention;

30 FIG. 2 is a cross-sectional view of the apparatus taken along line 2-2 in FIG. 1;

FIG. 3 is a perspective side view of a yarn plug produced by the process of the invention;

FIG. 4 is a sectional view of the yarn plug taken along line 4-4;

FIG. 5 is a schematic diagram of a process wherein the yarn is preheated before entering a yarn bulking device;

FIG. 6 is a schematic diagram of a process wherein a yarn is drawn before entering a yarn bulking device; and

FIG. 7 is a schematic diagram illustrating the embodiments of the process wherein the yarn is subjected to various treatments before entering the yarn bulking device.

#### DESCRIPTION OF THE PREFERRED EMBODIMENTS

In FIG. 1, nylon feeder yarn 1 is drawn from a pair of feed rollers or like feeding device into an aspirator jet unit, generally designated by reference numeral 2, through yarn inlet tube 3. Superheated steam is supplied to the aspirator jet unit by steam inlet pipe 4 and discharges into a temperature sensing zone 5 before passing through a narrow passage 6 of the jet nozzle 7 to the orifice 8.

The longitudinal axis of the yarn inlet tube is arranged at an angle of about 45° with the longitudinal axis of the jet and is positioned with an exit opening upstream of and closely adjacent to the jet orifice. Also, as shown in FIG. 2, the axis of the yarn inlet tube 3 and the axis of the passage 6 leading to the orifice 8 are in the same vertical plane.

Advantageously, it has been found that when the discharge end, i.e. the tip, of the jet nozzle is bent at an angle of from 2° to 8° from the longitudinal axis of the nozzle, the symmetry of the yarn plug, i.e. with respect to the arrangement of the filaments therein and unifor-

mity of its outer surface, is greatly improved. Furthermore, the top preferably should be bent towards the lower right-hand quadrant of the cross-section shown in FIG. 2, although advantageous effects are also obtained when the tip is bent towards the surrounding sectors that are circumscribed by an arc angle of 45° (the area to the right of line "a—a" in FIG. 2 defines the sectors wherein these results are obtained). It will be understood that the "tip" of the jet nozzle refers to about the last  $\frac{1}{8}$  inch of the nozzle.

It will be appreciated that it is generally preferred also to employ an external preheater means (not shown) such as a plate heater, heated godet, etc. that will heat the yarn to a temperature of from 150° C. - 200° C. before it enters the yarn inlet tube.

The feeder yarn is propelled or carried by the steam through the conically-shaped entrance 9 (having a convergent angle of about 60°) of the preheat tube 10 into passage 11 where the yarn is preheated by the superheated steam to a temperature between the second order transition point and the melting point of the yarn.

The yarn and steam then enter a diffuser 12 at the other end of tube 10 which is also provided with a conical wall 13. The angle of divergence of wall 13 may vary from about 20° to 60° and preferably is about 30°.

In the diffuser, the steam rapidly expands and causes the yarn to splay outwardly towards the surface of wall 13. The flat shoulder 14 at the end of the diffuser creates an eddy-effect to allow the yarn filaments to go onto a smooth wall portion 15 which defines the front end of 30 the bulking chamber 16 and then to fold inwardly against themselves thereby forming a compacted yarn mass. The yarn mass soon accumulates and forms an elongated plug that is pushed into an air permeable, e.g. slotted, wall portion 17 of the bulking chamber by the back pressure developed in the smooth side wall portion due to resistance of the steam flowing through the plug. A plurality of slots 17' are arranged uniformly around the periphery of the chamber. In the embodiment shown, 18 slots are provided in the tubular member 40 defining the bulking chamber. Reference numeral 18 generally designates the plug; whereas 18' refers to the initially formed yarn mass or plug; and reference numeral 18" designates the portion of the plug extending out of the slotted portion. It will be appreciated that the 45 tubular member forming the air permeable portion of the bulking chamber may be provided with perforations having different configurations, e.g. circular, which are arranged in various patterns to provide uniform escape of gas therefrom. Also, this portion of the chamber could be formed by convolutions of a coil or like wall construction having opening therein. Preferably a slotted tubular member, as shown, is employed since it provides guide strips between the slots that promote displacement of the plug with uniform escape of the 55 steam.

In the smooth side wall portion 15, all of the steam passes axially through the formed plug before discharging laterally through slots 17'. The steam exiting from the slots then collects in an exhaust chamber 19 surrounding the slotted portion of the bulking chamber. The steam is then discharged to the atmosphere or a collecting tank via exhaust pipe 20. A heat insulated shroud 21 surrounds the entire yarn bulking apparatus. Plug 18 is further pushed through a tubular conduit 22 to a take-up unit 23 in a manner similar to that described in the above-referenced Fink application. This unit includes a plug guide for positioning the end of the plug

as a yarn bundle is pulled from the plug by a take-up device for winding the yarn into a package.

In order to determine the temperature of the steam just prior to entering the jet nozzle a temperature sensing control 24 with a temperature probe 25 is provided. The temperature probe extends into zone 5 at substantially right angles to the steam entering through inlet pipe 4. A housing 26 is provided for the temperature probe. As heretofore described, the take-up device 10 withdraws the yarn at a rate which is about 15-25% less than the rate the yarn is introduced by the feed means. Both the take-up device and the feed means operate at substantially constant rates. Also, appropriate control means may be provided to allow for variations in the plug formation during operation of the apparatus. These controls have been described heretofore.

From the foregoing detailed description of the apparatus and process, it will be recognized that the present invention provides several advantages in texturizing the yarn. In particular, the smooth wall portion of the diffuser enables the yarn to fold upon itself to form a more uniform plug in that the filaments pack more uniformly to provide greater density and the smooth outer periphery of the plug allows it to pass more uniformly through the bulking chamber. Also, since the yarn filaments, which fold upon themselves on the smooth side wall portion of the bulking chamber, are generally arranged radially inward from the smooth side wall portion and at an angle to its longitudinal axis, when the plug moves forward due to the pressure exerted on it by the stream, the steam is allowed to exhaust through the slots in the slotted portion of the bulking chamber without causing the filaments of the yarn plug to pass into the slots.

Moreover, it is of considerable importance that all of the steam must pass through the initially formed portion of the plug. This results in a more uniform and effective steam heating and conditioning of the filaments in the folded and compacted state. Also, the steam and filaments carried by the steam more uniformly impinge on the initially formed yarn plug since the steam does not escape directly to the atmosphere but is controlled by being blown through at least the initially formed portion of the plug. Consequently, the crimps obtained in the filaments are more uniform and evenly distributed throughout.

Because the plug forms on a solid side wall portion of the bulking chamber and all steam passes forward through the plug at this stage of the process, a substantially greater pushing force (i.e. plug compacting force) is exerted on the front of the yarn plug. Consequently, the plug is less sensitive to stack-height variation and thereby permits longer plugs to be utilized without causing variations in the bulkiness and crimps of the yarn. Also, the aspirator jet is less subject to variations due to a change in back pressure since the plug can move forward and backward in the smooth side wall portion of the bulking chamber without changing the exhaust pattern of the steam through the slotted wall portion of the chamber.

It will also be appreciated that since there is a substantially large pushing force available for causing the plug to move forward, since the apparatus is less sensitive to moderate variations in the positioning of the initial plug portion and since all the steam is exhausted from the plug before the plug exits from the top of the slotted portion of the bulking chamber, the end or top of the plug is made available for contact with sensing devices such as microswitches, pneumatic sensors, pho-

toelectric sensors and the like for end-out detection and/or windup speed control. Also, the configuration of the yarn plug is more geometrically defined and has a firm outer periphery thereby enabling the plug to be sensed more easily by feeler type devices.

The process of the invention will be further understood from the following examples:

#### EXAMPLE 1

A nylon carpet yarn of 136 filaments with trilobal cross-section and a denier of 2,080 after being drawn to an approximate 4.0 draw ratio is taken from a creel and passed over a plate-type heater operated at 188° C. This yarn then enters the nip of two feed rollers and is nipped with sufficient force to pull the yarn across the pre-heater plate. From the feed rolls, the yarn is introduced into the yarn inlet tube of an apparatus of the type illustrated in FIGS. 1 and 2 of the drawings. This yarn is initially strung up by passing the feeder yarn through the apparatus to be received by an operator who secures the yarn to a take-up device, particularly a flat package take-up device. This take-up device operates at a take-up speed of approximately 835 meters per minute; whereas the feed rate is 980 meters per minute.

Simultaneously, with actuation of the take-up device 25 superheated steam at 235° C. and 75 psig, is introduced into the steam inlet pipe. The yarn is continuously drawn into the bulking apparatus to provide a yarn plug which is continuously forced out of the apparatus and then passed through a plug guide operatively associated 30 with the take-up device wherein a yarn bundle is continuously separated from the plug at a tension of up to about 5 grams by the take-up device.

The resulting yarn product was evaluated over a week's time and found to exhibit the following average 35 properties:

Bulked denier; 2759  
Strength (G/Den) 2.22  
Elongated (%) 58.3  
Bulk(%) 15  
Tangle Factor (100 in.) 217  
Crimp Count (1 in.) 13.0  
Shrinkage (%) 2.9  
Finish (%) 0.8

Also, evaluation of the plug revealed that the density 45 of the plug varied from a minimum of about 3.6 g/cu. in. to a maximum of about 3.75 g/cu. in.

#### EXAMPLE 2

Additional runs were conducted in which the same 50 feeder yarn as used in Example 1 as employed in the same apparatus to produce carpet yarns. Upon evaluation over a period of several weeks, it was found that the denier of the yarn varied from a low of 2722 to a high of 2803 and the average crimp count per inch varied from about 12 to about 14. Also, the other above-noted properties were found to be substantially uniform over this period and comparable to those obtained in Example 1. It will be apparent that these results establish that the process of the present invention provides an exceptionally uniform yarn product having excellent crimp. In all cases, the yarn was found to be substantially free of snarls and tangles.

#### EXAMPLE 3

Microscopic examination of the yarns produced in the foregoing Examples revealed that each of the filaments has a uniform degree of evenness and crimp and

that the crimp count throughout substantially all of the filaments of the yarn varied from 12 to 14, with occasional minute crunodal loops appearing in the filaments. These loops are removed from the yarn upon applying 5 a tension of about 80 grams

The configuration of the yarn plug or mass of compacted yarn produced by the process exemplified in the foregoing Examples is shown in FIGS. 3 and 4. It will be seen that the plug has a body with an elongated rod-like shape in which the filaments of the yarn are compacted in a dense arrangement. A major portion of the filaments have portions which extend at an angle to the axis of the plug as heretofore described with intermediate portions or sections of the filaments forming 15 alternate inwardly and outwardly curved folds or pleats. The appearance of this arrangement of the filaments is somewhat like that of an accordion. It will be noted that in FIG. 3, an end portion of the semi-rigid body of the plug has been broken away from the remaining portion of the plug to show the arrangement of the filaments.

As further shown in FIG. 3, the filaments when pulled from the plug in the form of a yarn bundle appear to converge together from points evenly distributed alternately at the center and then at the periphery of the plug. These filaments are elongated into the form of a yarn bundle without the occurrence of any snarls or tangles.

#### EXAMPLE 4

In order to further evaluate the luminosity of texturized yarn obtained by the process of this invention, additional experiments were conducted. In these experiments, sample lengths of yarn were passed through a sensing head of a G.E. "Qualigard" yarn monitoring device. In general use, the yarn sensing head of this device operates as a backpressure air gaging sensor which detects variations in yarn denier and converts the variations to a minute proportional air pressure.

In the following experiments, the sensing head was employed to provide a backpressure reading that is proportional to the luminosity of the texturized yarn. Air was supplied to a SHPAV with a constant pressure, i.e. 25 psig. This air enters the sensor slot at its midpoint and escapes through the slot at either end. A yarn passing through the sensor slot impedes the air flow and creates a backpressure proportional to the total effective cross-sectional area of the yarn. The backpressure is converted into a "Qualigard" reading in inches of water, a larger number for equivalent flat denier indicating a more luminous yarn.

The test apparatus used was a "Qualigard" Model CR 280 YM31A with sensing head No CR280 GP 11A060. 55 This test apparatus was calibrated by inserting a wire having a diameter of 0.0404 into the slot of the sensing head. The air supply to the sensing head pressure adjustment valve was adjusted to 25 psig, and the sensing head pressure adjustment valve was adjusted to read 14 inches of water. Then the yarn sample was passed through the sensor slot at a preset speed of 1 inch per sec. and a tension of 70 grams.

Samples of nylon yarn produced in accordance with the procedure outlined in Example 1 having actual 65 denier of 2700 (Sample A) and samples of nylon yarns (Samples B and C) having deniers comparable to Sample B, which are commercially available, were evaluated. The results of these tests are tabulated below:

| Yarn                                   | Qualigard Reading | Actual Denier |
|----------------------------------------|-------------------|---------------|
| A                                      | 35                | 2700          |
| B <sup>(1)</sup>                       | 22                | 2750          |
| C <sup>(2)</sup>                       | 23                | 2600          |
| (1) Product of Allied<br>MERGE 90026   |                   | (2750)        |
| (2) Product of DuPont<br>MERGE 13 828M |                   | (2600)        |

From the above data, it will be apparent that the 10  
texturized yarns of the invention are more voluminous  
than the comparable commercially available yarns.

The smooth tightly packed yarn plug produced by  
the process of this invention has a density from about  
three to four grams per cubic inch. The density and size  
of the plug are sufficient to permit the plug to be physi-  
cally handled or manipulated by a machine without any  
significant distortion. This permits numerous treatments  
to be made while the yarn is in this compact and slow  
moving geometry within the apparatus of the invention.

Advantageously, the surface of the yarn plug may  
also be cut to a shallow depth at spaced intervals around  
the periphery of the plug. In this manner, some but not  
all of the filaments in the resulting yarn bundle would be  
cut resulting in a fuzzy or staple-like yarn product.

It will be further appreciated that various anti-static  
and/or anti-soiling materials may be added to the yarn  
while it is retained in the bulk form by directly applying  
these materials to the plug. Also, additional heat-setting  
of the yarn can be effected while the yarn is in the plug  
form.

It will be appreciated that the dimensions of the vari-  
ous elements of the apparatus of the present invention  
may vary considerably while still providing the neces-  
sary passages for bulking of the yarn. Generally, the  
nozzle jet has a diameter that is equal to or approxi-  
mately one-half the diameter of the preheat tube. Also,  
the bulking chamber usually has a diameter of at least  
about seven times the diameter of the nozzle jet with a  
smooth wall portion of at least about one-half inch to  
insure the formation of a suitably sized plug. Moreover,  
the length of the entire bulking chamber usually varies  
from about three to ten times its diameter with the slots  
provided in the slotted wall portion each having a  
width from a few to several one hundreds of an inch.

It will be appreciated that at the higher operating  
pressures, e.g. at 70 psig. or above, the aspirating effect  
that occurs at the yarn inlet of the jet means is no longer  
apparent, i.e. the pressure goes from negative to positive  
during the bulking operation.

While the novel embodiments of the invention have  
been described, it will be understood that various omis-  
sions, modifications and changes in these embodiments  
may be made by one skilled in the art without departing  
from the spirit and scope of the invention.

What we claim is:

1. A process for texturizing yarn which comprises:  
passing a synthetic polymeric multifilament yarn  
together with a stream of heated gas into a diverg-  
ing conical diffuser zone to cause the gas stream to  
rapidly expand and to cause the filaments of the  
yarn to splay outwardly from the center of the  
expanding gas stream;  
creating an eddy-effect at the end of the diffuser zone  
to cause yarn filaments splayed outwardly in said  
diffuser zone to contact a smooth imperforate con-  
tinuous wall portion of such length as to insure the  
formation of a compacted yarn mass therein and

- said smooth wall portion defining an upstream end  
of a bulking chamber;  
forming the yarn filaments into a compacted yarn  
mass within said smooth wall portion at said up-  
stream end of the bulking chamber;  
pushing the compacted yarn mass into and through  
an air permeable wall portion of the bulking cham-  
ber while the gas initially passes through the com-  
pacted yarn mass at said upstream end of the cham-  
ber; and subsequently discharges laterally from the  
yarn mass within the air permeable wall portion of  
the bulking chamber; and  
withdrawing a yarn bundle from the compacted yarn  
mass.
2. The process of claim 1, wherein said yarn is pre-  
heated to a temperature from about 100° C. to 200° C.  
before entering the gas stream.
  3. The process of claim 1, wherein said gas stream is  
formed by an aspirator jet and the yarn is pulled into  
said gas stream by a venturi effect created by said aspi-  
rator jet.
  4. The process of claim 3, wherein said yarn is drawn  
at a draw ratio of from 2.5 : 1 to 4 : 1 before entering said  
aspirator jet.
  5. The process of claim 3, wherein said yarn is spun,  
packaged and then drawn before entering said aspirator  
jet.
  6. The process of claim 3, wherein said yarn is spun-  
drawn before entering said aspirator jet.
  7. The process of claim 3, wherein yarn is spun-drawn  
and then packaged before entering said aspirator jet.
  8. The process of claim 1, wherein said gas is super-  
heated stream at a temperature of from 200° C. to 275°  
C. and a pressure of from 50 to 100 psig.
  9. The process of claim 1, wherein said gas is com-  
pressed air at a pressure of from 50 to 100 psig. and a  
temperature of from 200° to 275° C.
  10. The process of claim 1, wherein all the gas exiting  
from said diffuser zone passes through an initially  
formed portion of said yarn mass located in said smooth  
wall portion of the bulking chamber and the gas passed  
therethrough discharges laterally from said mass  
through slots formed in the air permeable wall portion  
of said bulking chamber.
  11. The process of claim 1, wherein the yarn is fed to  
said diffuser at a constant rate and a yarn bundle is  
withdrawn from the yarn mass at a rate that is about  
15-25% less than said constant feed rate.
  12. The process of claim 1, wherein said synthetic  
polymeric yarn is a nylon yarn.
  13. In a continuous process for the texturizing of yarn  
in a gas jet bulking process wherein the yarn is aspirated  
along with a heated gas into a yarn bulking chamber,  
the improvement comprising:  
passing the yarn together with the stream of heated  
gas into a diverging conical diffuser zone to cause  
the gas stream to expand rapidly and to cause the  
filaments of the yarn to splay open;  
creating an eddy-effect at the end of the diffuser zone  
to cause yarn filaments splayed open to contact a  
first tubular smooth imperforate wall zone of the  
bulking chamber of such a length to insure the  
formation of a compacted yarn plug therein;  
forming a compacted yarn plug from an initial length  
of yarn filaments within said first tubular smooth  
imperforate wall zone, the upstream face of the

**13**

plug being concave toward the downstream end of the plug;  
impinging successive yarn filaments in a controlled random oscillatory manner on the formed plug 5 surface while passing the heated gas axially

**14**

through at least the initially formed portion of the plug within said smooth wall zone; pushing the yarn plug into and through a second perforate wall portion of the bulking chamber; and withdrawing a yarn bundle from the yarn plug.

\* \* \* \* \*

10

15

20

25

30

35

40

45

50

55

60

65